

# UNITED STATES PATENT OFFICE.

RALPH H. MCKEE, OF RIDGEFIELD PARK, NEW JERSEY.

## FIXATION OF NITROGEN.

1,236,853.

Specification of Letters Patent. Patented Aug. 14, 1917.

No Drawing.

Application filed October 26, 1916. Serial No. 127,959.

To all whom it may concern:

Be it known that I, RALPH H. MCKEE, a citizen of the United States, residing at Ridgefield Park, in the county of Bergen 5 and State of New Jersey, have invented certain new and useful Improvements in the Fixation of Nitrogen, of which the following is a specification.

It is known that free nitrogen may be caused to enter into combination (fixed) by 10 passing nitrogen or air in contact with a mixture containing an alkali metal or its carbonate, carbon, and a suitable metal or metal oxid reducible by carbon, the mixture being maintained at a high temperature, say 15 1,000° C., more or less, during the process. A typical case of the above reaction is the passage of nitrogen over a highly heated mixture consisting of about two parts of coke, two parts of iron oxid, and one part 20 of soda-ash. This charge is placed in containers, to which heat is applied in any suitable way.

Charge containers for use in the above process have heretofore been made of iron, but these have not proven satisfactory in practice, for the reasons among others that they are quickly destroyed under the very severe working conditions, and moreover, 25 exert a decomposing action upon the sodium or potassium cyanid which is initially formed.

I have discovered that excellent results are obtained in carrying out processes of 30 the type above described, by the use of charge containers formed of an alloy consisting principally or essentially of nickel, chromium, and iron. For the best results this alloy should contain at least 50 per 35 cent. of nickel, 10 to 20 per cent. of chromium, 10 to 30 per cent. of iron, less than 10 per cent. of manganese, and less than two per cent. of carbon. A typical alloy may contain nickel, 60 per cent.; chromium, 12 40 per cent.; iron, 25 per cent.; manganese, three per cent.; with usually a small proportion, less than one per cent., of carbon.

The containers will in the simplest case 45 take the form of round or flattened tubes or 50 pipes, although any suitable forms may be

used. The vessels may be either cast, rolled or drawn from the proper alloy composition. External application of heat is simplest, although internal (electrical) heating may be used. When metallic sodium is used, preferably in the form of vapor, the reaction is exothermic; whereas with soda-ash the reaction is strongly endothermic.

The alloys above described possess in this particular process the following important 60 technical advantages:—

(1) The containers are durable and resistant, being entirely serviceable under the very severe industrial conditions of the process.

(2) The composition of the container 65 appears to exert a direct and favorable influence upon the rate of the reaction. This is presumably due to the fact that the rate of this particular reaction is favorably catalyzed by both nickel and chromium, which 70 are present in the exposed interior walls of the container.

I claim:—

1. In a nitrogen-fixation process of the character set forth, the step which consists 75 in effecting the reaction in a container having exposed interior walls of an alloy containing nickel, chromium and iron.

2. In a nitrogen-fixation process of the character set forth, the step which consists 80 in effecting the reaction in a container having exposed interior walls of an alloy containing at least 50 per cent. of nickel, 10 to 20 per cent. of chromium, and 10 to 30 per cent. of iron.

3. In a nitrogen-fixation process of the character set forth, the step which consists 85 in effecting the reaction in a container having exposed interior walls of an alloy containing approximately 60 per cent. of nickel, 90 12 per cent. of chromium, 25 per cent. of iron, and small proportions of manganese and carbon.

In testimony whereof I affix my signature in presence of two witnesses.

RALPH H. MCKEE.

Witnesses:

EDMOND F. WRIGHT,  
F. W. SCHELLMAN.